



US009764384B2

(12) **United States Patent**  
**Mittendorf et al.**

(10) **Patent No.:** **US 9,764,384 B2**  
(45) **Date of Patent:** **Sep. 19, 2017**

(54) **METHODS OF PRODUCING DISPERSOID HARDEDENED METALLIC MATERIALS**

(71) Applicant: **HONEYWELL INTERNATIONAL INC.**, Morristown, NJ (US)

(72) Inventors: **Don Mittendorf**, Mesa, AZ (US);  
**Vladimir K. Tolpygo**, Scottsdale, AZ (US)

(73) Assignee: **HONEYWELL INTERNATIONAL INC.**, Morris Plains, NJ (US)

(\*) Notice: Subject to any disclaimer, the term of this patent is extended or adjusted under 35 U.S.C. 154(b) by 274 days.

(21) Appl. No.: **14/686,313**

(22) Filed: **Apr. 14, 2015**

(65) **Prior Publication Data**

US 2016/0303653 A1 Oct. 20, 2016

(51) **Int. Cl.**

*C22C 1/04* (2006.01)  
*B22F 1/00* (2006.01)

(Continued)

(52) **U.S. Cl.**

CPC ..... *B22F 1/0081* (2013.01); *B22F 1/0003* (2013.01); *B22F 1/0085* (2013.01);  
(Continued)

(58) **Field of Classification Search**

None

See application file for complete search history.

(56)

**References Cited**

U.S. PATENT DOCUMENTS

3,753,795 A \* 8/1973 Weber ..... C22C 32/0026  
148/410  
3,779,714 A 12/1973 Nadkarni et al.

(Continued)

FOREIGN PATENT DOCUMENTS

DE 2262132 A1 6/1974  
WO 2015001241 A2 1/2015

OTHER PUBLICATIONS

Bestor, M.A., et al; Influences of chromium and hafnium additions on the microstructures of b-nial coatings on superalloy substrates; *Intermetallics* 19 (2011) 1693e1704; The University of Alabama, Department of Metallurgical and Materials Engineering; journal homepage: [www.elsevier.com/locate/intemet](http://www.elsevier.com/locate/intemet).

(Continued)

*Primary Examiner* — George Wyszomierski

(74) *Attorney, Agent, or Firm* — Lorenz & Kopf, LLP

(57) **ABSTRACT**

Methods of forming dispersoid hardened metallic materials are provided. In an exemplary embodiment, a method of producing dispersoid hardened metallic materials includes forming a starting composition with a base metal component and a dispersoid forming component. The starting composition includes the base metal component in an amount from about 50 to about 99.999 weight percent and the dispersoid forming component in an amount from about 0.001 to about 1 weight percent, based on the total weight of the starting composition. A starting powder is formed from the starting composition, and the starting powder is fluidized with a fluidizing gas for a period of time sufficient to oxidize the dispersoid forming component to form the dispersoid hardened metallic material. The dispersoid forming component is oxidized while the starting powder is a solid.

**20 Claims, 1 Drawing Sheet**



|      |                   |                                                                                                                                                                                |  |              |    |                         |
|------|-------------------|--------------------------------------------------------------------------------------------------------------------------------------------------------------------------------|--|--------------|----|-------------------------|
| (51) | <b>Int. Cl.</b>   |                                                                                                                                                                                |  |              |    |                         |
|      | <i>C22C 1/05</i>  | (2006.01)                                                                                                                                                                      |  | 8,748,008    | B2 | 6/2014 Chun et al.      |
|      | <i>C22C 1/10</i>  | (2006.01)                                                                                                                                                                      |  | 2008/0142126 | A1 | 6/2008 Gigliotti et al. |
|      | <i>C22C 32/00</i> | (2006.01)                                                                                                                                                                      |  | 2009/0123690 | A1 | 5/2009 Scholl et al.    |
|      | <i>B22F 1/02</i>  | (2006.01)                                                                                                                                                                      |  | 2010/0279146 | A1 | 11/2010 Rowe et al.     |
|      | <i>B22F 9/16</i>  | (2006.01)                                                                                                                                                                      |  | 2012/0244456 | A1 | 9/2012 Muecke et al.    |
| (52) | <b>U.S. Cl.</b>   |                                                                                                                                                                                |  | 2013/0255843 | A1 | 10/2013 Kiuchi et al.   |
|      | CPC .....         | <i>B22F 1/02</i> (2013.01); <i>B22F 9/16</i> (2013.01); <i>C22C 1/056</i> (2013.01); <i>C22C 1/1036</i> (2013.01); <i>C22C 1/1068</i> (2013.01); <i>C22C 32/0026</i> (2013.01) |  | 2014/0294653 | A1 | 10/2014 Kim et al.      |
|      |                   |                                                                                                                                                                                |  | 2015/0027993 | A1 | 1/2015 Bruck et al.     |

(56) **References Cited**

## U.S. PATENT DOCUMENTS

|               |         |                  |              |        |
|---------------|---------|------------------|--------------|--------|
| 3,992,161 A * | 11/1976 | Cairns .....     | C22C 32/0026 |        |
|               |         |                  |              | 75/234 |
| 5,429,793 A   | 7/1995  | Ong et al.       |              |        |
| 5,480,468 A   | 1/1996  | Ritter et al.    |              |        |
| 5,510,080 A   | 4/1996  | Nishi et al.     |              |        |
| 5,571,304 A   | 11/1996 | Ritter et al.    |              |        |
| 5,989,491 A   | 11/1999 | Isomoto et al.   |              |        |
| 6,143,241 A   | 11/2000 | Hajaligol et al. |              |        |
| 6,168,871 B1  | 1/2001  | Ritter et al.    |              |        |
| 6,485,584 B1  | 11/2002 | Lambard et al.   |              |        |
| 6,893,481 B2  | 5/2005  | Nam et al.       |              |        |
| 7,361,235 B2  | 4/2008  | Ohtsuka et al.   |              |        |
| 7,699,905 B1  | 4/2010  | Anderson et al.  |              |        |
| 8,313,810 B2  | 11/2012 | Helmick et al.   |              |        |
| 8,603,213 B1  | 12/2013 | Anderson et al.  |              |        |

## OTHER PUBLICATIONS

Humbert, M.; Oxide Dispersion Strengthened Alloys; 3.40 Dec. 17, 2012; Reference Notes available online at <http://li.mit.edu/Stuff/PM/Termpaper/MattHumbert-termpaper.pdf>.

Li, D, et al.; Cyclic oxidation of b-NiAl with various reactive element dopants at 1200 C; Corrosion Science 66 (2013) 125-135; School of Materials Science and Engineering, Beihang University, No. 37, Beijing Key Laboratory for Advanced Functional Material and Thin Film Technology, Beihang University, No. 37; journal homepage: [www.elsevier.com/locate/corsci](http://www.elsevier.com/locate/corsci).

Ohtsuka, S. et al.; High temperature reaction tests between high-Cr ODS ferritic steels and U—Zr metallic fuel; Journal of Nuclear Materials 441 (2013) 286-292; Advanced Nuclear System R&D Directorate, Japan Atomic Energy Agency, Graduate School of Engineering, Hokkaido University, Kobelco Research Institute, Japan, Institute of Advanced Energy, Kyoto University; journal homepage: [www.elsevier.com/locate/jnucmat](http://www.elsevier.com/locate/jnucmat).  
Extended EP Search Report for Application No. 16163946.3-1373 dated Jul. 29, 2016.

\* cited by examiner



## METHODS OF PRODUCING DISPERSOID HARDEDEN METALLIC MATERIALS

### TECHNICAL FIELD

The present disclosure generally relates to methods of forming dispersoid hardened metallic materials, and more particularly relates to methods of forming dispersoids in metallic powders in solid form.

### BACKGROUND

Many metals can be hardened by including dispersoids within a matrix of the metal. Dispersoid strengthened metallic materials include a metal matrix, which may be an alloy, with dispersoids distributed throughout the matrix. Dispersoids are typically oxides of a metallic component, where the metallic component that is oxidized is different than the bulk of the metal material. The dispersoids increase the strength and hardness of the metallic matrix. Dispersoid hardened metallic materials have been formed mechanically, where a dispersoid (such as yttrium oxide ( $Y_2O_3$ )) is extensively milled and then blended with a base metal component, such as iron (Fe) and chromium (Cr) powders. The milling and blending process may proceed for days to produce the desired product, in part because the desired size of the dispersoids is quite small, such as 1 micron or less. After milling and blending, thermo-mechanical treatments may be used for secondary recrystallization that can produce a stronger microstructure. The thermo-mechanical treatment may be hot rolling with high temperature treatment, for example, but other treatments are also possible. The cost to mechanically produce dispersoid hardened metallic materials is prohibitive, and this high cost has prevented widespread use of dispersoid hardened metallic materials.

Accordingly, it is desirable to provide methods for producing dispersoid hardened metallic materials that are economically viable. In addition, it is desirable to provide methods of forming dispersoid hardened metallic materials in a reasonable time period, where the dispersoids have a particle size of about 1 micron or less. Furthermore, other desirable features and characteristics of the present embodiment will become apparent from the subsequent detailed description and the appended claims, taken in conjunction with the accompanying drawings and this background of the invention.

### BRIEF SUMMARY

Methods of forming dispersoid hardened metallic materials are provided. In an exemplary embodiment, a method of producing dispersoid hardened metallic materials includes forming a starting composition with a base metal component and a dispersoid forming component. The starting composition includes the base metal component in an amount from about 50 to about 99.999 weight percent and the dispersoid forming component in an amount from about 0.001 to about 1 weight percent, based on the total weight of the starting composition. A starting powder is formed from the starting composition, and the starting powder is fluidized with a fluidizing gas for a period of time sufficient to oxidize the dispersoid forming component to form the dispersoid hardened metallic material. The dispersoid forming component is oxidized while the starting powder is a solid.

A method for forming dispersoid hardened metallic materials is provided in another embodiment. The method includes forming a starting composition with a base metal

component and a dispersoid forming component. The base metal component is from about 50 to about 99.999 weight percent of the starting composition, and the dispersoid forming component is from about 0.001 to about 1 weight percent of the starting composition. A starting powder is formed from the starting composition, where the starting powder includes starting particulates. An oxidizing agent is diffused into the starting particulates while in a solid state, and the dispersoid forming component is oxidized within the starting particulates while in the solid state to form the dispersoid hardened metallic material.

A method for forming dispersoid hardened metallic materials is provided in yet another embodiment. The method includes forming a starting composition with a base metal component and a dispersoid forming component. The base metal component is from about 50 to about 99.999 weight percent of the starting composition, and the dispersoid forming component is from about 0.001 to about 1 weight percent of the starting composition. About 50 weight percent or more of the dispersoid forming component within the starting composition is preferentially oxidized while the starting composition is in a solid state, and about 95 weight percent or more of the base metal component is present in a reduced state.

### BRIEF DESCRIPTION OF THE DRAWINGS

Various embodiments will hereinafter be described in conjunction with the FIGURE, which is a schematic diagram of an exemplary embodiment of an apparatus and method for producing dispersoid hardened metallic materials.

### DETAILED DESCRIPTION

The following detailed description is merely exemplary in nature and is not intended to limit the various embodiments or the application and uses of the invention. Furthermore, there is no intention to be bound by any expressed or implied theory presented in the preceding technical field, background, brief summary, or the following detailed description.

Referring to the FIGURE, a method for producing a dispersoid hardened metallic material **10** is provided in accordance with an exemplary embodiment. In this description, a “metallic material” is a material that has the physical properties of a metal, and wherein a majority of the chemical bonds in the metallic material are metallic bonds. As such, a metallic material may include metalloids or non-metals, as long as the metallic properties and metallic bonding are present. The method includes providing a starting composition **12** that includes a base metal component **14**, a dispersoid forming component **16**, and optionally an alloy material **18**, all of which are in a reduced state. The base metal component **14** is a metallic material that forms about 50% or more of the starting composition **12**. As used herein, the term “reduced state” means a small percentage or no oxide-bound material of the composition is present, such that about 0 up to a maximum of about 10 weight percent of the material is chemically bound to an oxygen atom. In an exemplary embodiment, the base metal component **14** consists of nickel (Ni), cobalt (Co), iron (Fe), copper (Cu), or a combination thereof, and the base metal component **14** is present in the starting composition **12** at from about 50 to about 99.999 weight percent, where the weight percent is based on the total weight of the starting composition **12**. In alternate embodiments, the base metal component **14** is

present in the starting composition **12** at from about 60 to about 99.999 weight percent, or about 70 to about 99.999 weight percent. The starting composition **12** may also include oxides of the materials within the base metal component **14** at low concentrations, such as from about 0 to about 10 weight percent, or from about 0.001 to about 10 weight percent, or from about 0.001 to about 5 weight percent in various embodiments. The starting composition **12** also includes a dispersoid forming component **16** at from about 1 to about 0.001 weight percent, or at from about 0.5 to about 0.001 weight percent, or at from about 0.2 to about 0.001 weight percent in various embodiments.

The dispersoid forming component **16** includes an element that is more easily oxidized than the base metal component **14**. In an exemplary embodiment, the dispersoid forming component **16** may include a metal that is as easy or easier to oxidize than aluminum. For example, the dispersoid forming component **16** may be selected from the group consisting of hafnium, zirconium, yttrium, scandium, lanthanum, cerium, praseodymium, neodymium, promethium, samarium, europium, gadolinium, terbium, dysprosium, holmium, erbium, thulium, ytterbium, lutetium, and combinations thereof. In an alternate embodiment, the dispersoid forming component **16** includes aluminum. In yet another embodiment, the dispersoid forming component **16** is selected from the group consisting of hafnium, zirconium, and yttrium. As with the base metal component **14**, oxides of the dispersoid forming component **16** may be present in the starting composition **12** at low concentrations, such as from about 0 to about 0.1 weight percent, or from 0.0001 to about 0.1 weight percent, or from about 0.0001 to about 0.01 weight percent in various embodiments.

The starting composition **12** may optionally include an alloy material **18** at from about 0 to about 50 weight percent, where the alloy material **18** may be almost any compound. As used herein, the term “alloy” means a metallic material formed with the base metal component **14** and one or more alloy materials **18**, where the alloy has one or more improved properties over the base metal component **14**. In alternate embodiments, the alloy material **18** is present in the starting composition **12** at from about 5 to about 50 weight percent, or from about 10 to about 40 weight percent, or from about 10 to about 30 weight percent. The starting composition **12** may also include other compounds in some embodiments, such as carbon or impurities. The dispersoid forming component **16** is also more easily oxidized than the alloy material **18**, in embodiments where an alloy material **18** is present. The dispersoid forming component **16**, the base metal component **14**, and the optional alloy material **18** are selected such that the dispersoid forming component **16** is more easily oxidized than either of the base metal component **14** or the alloy material **18**, so the selection of the base metal component **14** and the alloy material **18** may influence the selection of the dispersoid forming component **16**. For example, if the alloy material **18** is aluminum, the dispersoid forming component **16** is a material that is more easily oxidized than aluminum. However, if the base metal component **14** and the alloy material **18** are both more resistant to oxidizing than aluminum, then the dispersoid forming component **16** may include aluminum.

The components of the starting composition **12** may be combined and melted to form a melt, so the components of the starting composition **12** can be thorough mixed. For example, the molten starting composition **12** may be mixed with an impeller **20**, as illustrated, but many other mixing techniques may also be used, including but not limited to a magnetic mixing bar, a static mixer, or simple addition

where combining and pouring the material provides adequate mixing. In an alternate embodiment, the components of the starting composition **12** may be combined and mixed as a powder, or the starting composition **12** may be acquired with the various components already present, such as from a recycling process, so no additional mixing is required.

In some embodiments, the starting composition **12** is formed into a starting powder **22**, where the starting powder **22** includes a plurality of starting particulates **24**. The starting composition **12** may be formed into the starting powder **22** in a wide variety of manners, including but not limited to crushing (as illustrated) and atomizing. Many apparatuses are available for crushing the starting composition **12**, such as hammer mills, ball mills, rollers, etc., and the starting composition **12** may be formed into a sponge-like material or other forms conducive to powder formation prior to the crushing process. In an alternate embodiment, liquid starting composition **12** is formed into small droplets and rapidly frozen to form the starting powder **22**, such as by exposing a small stream of molten starting composition **12** to high energy gaseous or liquid jets. Other options are possible for forming the starting composition **12** into the starting powder **22**. In an exemplary embodiment, the starting particulates **24** of the starting powder **22** have an average particle size of about 50 microns or less, or about 30 microns or less, or about 10 microns or less in various embodiments, where the average particle size is the D<sub>50</sub> particle size, or the median value of the particle size distribution. The starting powder **22** may be passed through a screen such that starting particulates **24** larger than the desired size are excluded. The larger particles may then be reprocessed and reduced in size, disposed of, or otherwise used. The shape of the starting particulates **24** is not critical.

The dispersoid forming component **16**, the base metal component **14**, and any other components of the starting composition **12** are randomly distributed within the starting particulates **24**, because the various components were evenly mixed and distributed within the starting composition **12** before it was formed into a powder.

The dispersoid forming component **16** is preferentially oxidized to form a dispersoid within the starting particulates **24**, while little to none of the base metal component **14** and the optional alloy material **18** are oxidized. In an exemplary embodiment, about 50 weight percent or more of the dispersoid forming component **16** is oxidized while about 95 weight percent or more of the base metal component **14** and about 95 weight percent or more of the alloy material **18** (if present) are present in the reduced state. In alternate embodiments, about 40 weight percent or more of the dispersoid forming component **16** is oxidized while about 95 weight percent or more of the base metal component **14** and about 95 weight percent or more of the alloy material **18** (if present) are present in the reduced state, or about 30 weight percent or more of the dispersoid forming component **16** is oxidized while about 95 weight percent or more of the base metal component **14** and about 95 weight percent or more of the alloy material **18** (if present) are present in the reduced state. The dispersoid forming component **16** is oxidized with an oxidizing agent, such as oxygen, carbon monoxide, water, or other materials that include oxygen. Without being bound by any particular theory, it is believed that the oxidizing agent oxidizes the dispersoid forming component **16** on the surface of the starting particulates **24**, and the oxidizing agent diffuses into the starting particulates **24** and oxidizes some or all of the dispersoid forming component **16** positioned within the interior of the starting particulates **24**. In an

exemplary embodiment, to preferentially oxidize the dispersoid forming component **16**, the starting powder **22** is fluidized with a fluidizing gas **26** for a period of time sufficient to oxidize the dispersoid forming component **16**, where the fluidizing gas **26** includes the oxidizing agent. As such, the oxidizing agent is external to the starting particulates **24** prior to exposure to the fluidizing gas **26**, so the oxidizing agent must diffuse into the starting particulates **24** to oxide much of the dispersoid forming component **16**. The fluidizing gas **26** may also include an inert component, such as nitrogen, argon, helium, etc. In many embodiments, the majority of the fluidizing gas **26** is inert.

The particle size of the starting particulates **24** may be selected such that the oxidizing agent is capable of diffusing into the starting particulates **24** within a reasonable period of time at the oxidizing conditions employed. Therefore, the particle size may vary for different compositions of the starting composition **12**, because different compositions may have different diffusivities at the oxidizing conditions in use. In some embodiments, the oxidizing agent may not diffuse to the core of the starting particulates **24**, so some of the dispersoid forming component **16** may remain in a reduced state. The low concentrations of dispersoid forming component **16** in a reduced state generally does not impair the properties of the final product, and a majority of the dispersoid forming component **16** is generally oxidized to form dispersoids.

The starting particulates **24** are in the solid state while the dispersoid forming component **16** is oxidized. The starting powder **22** is maintained at an oxidizing temperature, or within an oxidizing temperature range, while the dispersoid forming component **16** is oxidized. The oxidizing temperature is below the melting point of the base metal component **14**, and the starting particulates **24** remain in the solid state while the dispersoid forming component **16** is oxidized. In an exemplary embodiment, the oxidizing temperature is below the solidus temperature of starting composition **12**. If the oxidizing temperature were at or above the melting point of the base metal component **14**, some or all of the starting powder **22** may melt during the oxidation of the dispersoid forming component **16**. If the starting powder **22** melts, the dispersoid forming component **16** may tend to agglomerate or grow in size, which produces larger dispersoids. Smaller dispersoids are generally desired, so the oxidizing temperature is kept below the melting point of the base metal component **14** to limit agglomeration. As such, the average particle size (D50, as described above) of the dispersoids formed is about 1 micron or less, or about 0.5 microns or less, or about 0.3 microns or less in various embodiments. If the starting particulates **24** were liquid (i.e., liquid droplets of the starting composition **12**), the different components may tend to segregate somewhat, such as due to varying densities resulting in denser material accumulating near the outer surface of the starting particulates **24** due to centrifugal force from spinning. Other properties may also cause segregation of the components, such as different electronegativity, etc. However, since the starting particulates **24** are maintained in the solid state, the position of the dispersoid forming component **16** remains random, so the resulting dispersoids remains random within the dispersoid hardened metallic material **10**.

In some embodiments, there is a migration temperature below the melting point of the starting composition **12** where the dispersoid forming component **16** begins to migrate within a starting particulates **24** before the bulk of the starting particulates **24** melts. In such a case, the dispersoid forming component **16** may agglomerate somewhat,

which produces larger dispersoids. Therefore, the oxidizing temperature may be controlled at less than the migration temperature where the dispersoid forming component **16** becomes mobile within the starting powder **22**, such as about 10° C. below the melting point of the base metal component **14** or the alloy material **18** with the lowest melting point.

The oxidizing agent within the fluidizing gas **26** is present at a partial pressure that aids in selectively oxidizing the dispersoid forming component **16** over the base metal component **14** or the alloy material **18**. Thermodynamic principles can aid in selecting an oxidizing temperature and a partial pressure of the oxidizing agent that will oxidize the dispersoid forming component **16** while minimizing the oxidation of either the base metal component **14** or the alloy material **18**. Such thermodynamic principles can be calculated, and are readily available in many embodiments, such as Ellingham diagrams. Higher oxidizing temperatures and the higher partial pressures of the oxidizing agent can increase the rate of oxidation of the dispersoid forming component **16**, but higher oxidizing temperatures and partial pressures of the oxidizing agent also increase the likelihood of oxidation of the base metal component **14** and/or an alloy material **18**. As such, the oxidizing temperature and partial pressure of the oxidizing agent are selected to provide good selectivity to oxidize the dispersoid forming component **16** over the base metal component **14** and the alloy material **18**, and this is balanced with providing a favorable rate of oxidation of the dispersoid forming component **16**. In an exemplary embodiment, the oxidizing temperature influences the movement of the oxidizing agent into the starting particles **24**, as well as influencing the oxidizing selectivity of the dispersoid forming component **16** and the base metal component **14**. The oxidizing temperature may be selected to provide sufficient oxidizing agent movement within the starting particles **24** such that about 50 weight percent or more of the dispersoid forming component **16** is oxidized within about 16 hours or less while about 95 weight percent or more of the base metal component **14** and about 95 weight percent or more of the alloy material **18** (if present) are present in the reduced state.

Oxidation of the dispersoid forming component **16** to form the dispersoids converts the starting powder **22** into the dispersoid hardened metallic material **10**. The dispersoid hardened metallic material **10** is collected, and may be kept below the melting point of the dispersoid hardened metallic material **10** to prevent any agglomeration or segregation of components. The dispersoid hardened metallic material **10** in the powder form can be used in a wide variety of manners. For example, the powdered dispersoid hardened metallic material **10** can be formed into an article by a wide variety of methods, such as forging, sintering and forging, extrusion, three dimensional printing (such as direct metal laser sintering, direct metal laser melting, electron beam printing, etc.), plasma spraying, cladding, etc. The dispersoids remain randomly positioned within the dispersoid hardened metallic material **10**, so an article formed by extrusion or other methods may not have any directionality in its properties. Extrusion often produces an article with different shear strengths, hardness, or other properties in different directions, such as parallel with the axis of extrusion compared to perpendicular to the axis of extrusion. The random nature of the dispersoid positioning may avoid directional aspects of the article properties formed from the dispersoid hardened metallic material **10**.

While at least one embodiment has been presented in the foregoing detailed description of the invention, it should be appreciated that a vast number of variations exist. It should

also be appreciated that the embodiment or embodiments are only examples, and are not intended to limit the scope, applicability, or configuration in any way. Rather, the foregoing detailed description will provide those skilled in the art with a convenient road map for implementing an embodiment, it being understood that various changes may be made in the function and arrangement of elements described without departing from the scope as set forth in the appended claims and their legal equivalents.

What is claimed is:

1. A method of forming a dispersoid hardened metallic material comprising:

forming a starting composition comprising a base metal component and a dispersoid forming component, wherein the starting composition comprises the base metal component in an amount of from about 50 weight percent to about 99.999 weight percent and the dispersoid forming component in an amount from about 0.001 weight percent to about 1 weight percent based on the total weight of the starting composition;

20 forming a starting powder from the starting composition; fluidizing the starting powder with a fluidizing gas for a period of time sufficient to oxidize the dispersoid forming component within the starting powder and to form the dispersoid hardened metallic material, wherein the dispersoid forming component is oxidized while the starting powder is a solid.

2. The method of claim 1 wherein fluidizing the starting powder comprises fluidizing the starting powder at an oxidizing temperature for a period of time sufficient to oxide about 50 weight percent or more of the dispersoid forming component while about 95 weight percent or more of the base metal component is present in a reduced state, wherein the fluidizing gas is at an oxidizing temperature below a melting point of the base metal component.

3. The method of claim 1 wherein forming the starting composition comprises forming the starting composition with the base metal component, wherein the base metal component is selected from the group consisting of nickel, cobalt, iron, copper, or a combination thereof.

4. The method of claim 1 wherein forming the starting composition comprises forming the starting composition comprising an alloy material.

5. The method of claim 1 wherein forming the starting composition comprises forming the starting composition with the dispersoid forming component, wherein the dispersoid forming component has an affinity to oxygen greater than or equal to that of aluminum.

6. The method of claim 1 wherein forming the starting composition comprises forming the starting composition with the dispersoid forming component, wherein the dispersoid forming component is selected from the group consisting of hafnium, zirconium, yttrium, scandium, lanthanum, cerium, praseodymium, neodymium, promethium, samarium, europium, gadolinium, terbium, dysprosium, holmium, erbium, thulium, ytterbium, lutetium, and a combination thereof.

7. The method of claim 1 wherein oxidizing the dispersoid forming component comprises selecting an oxidizing temperature and an oxidizing agent partial pressure such that about 30 weight percent or more of the dispersoid forming component is oxidized and about 95 weight percent or more of the base metal component is in a reduced state.

8. The method of claim 7 wherein selecting the oxidizing temperature comprises selecting the oxidizing temperature such that about 50 weight percent or more of the dispersoid forming component is oxidized within about 16 hours or less

while about 95 weight percent or more of the base metal component is in the reduced state.

9. The method of claim 1 wherein oxidizing the dispersoid forming component comprises forming a plurality of dispersoids, wherein about 95 weight percent or more of the plurality of dispersoids have an average particle size of about 1 micron or less.

10. The method of claim 1 wherein oxidizing the dispersoid forming component comprises forming a plurality of dispersoids, wherein the plurality of dispersoids are randomly positioned within the dispersoid hardened metallic material.

11. A method of forming a dispersoid hardened metallic material comprising:

15 forming a starting composition comprising a base metal component and a dispersoid forming component, wherein the base metal component comprises from about 50 weight percent to about 99.999 weight percent of the starting composition and the dispersoid forming component comprises from about 0.001 weight percent to about 1 weight percent of the starting composition; forming a starting powder from the starting composition, wherein the starting powder comprises starting particulates; fluidizing the starting powder with a fluidizing gas; diffusing an oxidizing agent into the starting particulates while fluidizing the starting powder, wherein the oxidizing agent is within the fluidizing gas, and where the oxidizing agent is diffused into the starting particles while the starting particulates are in a solid state; and oxidizing the dispersoid forming component within the starting particulates with the oxidizing agent while the starting particulates are in the solid state to form the dispersoid hardened metallic material.

35 12. The method of claim 11 wherein forming the starting powder comprises forming the starting particulates with an average particle size of about 50 microns or less.

13. The method of claim 11 wherein oxidizing the dispersoid forming component within the starting particulates comprises oxidizing about 50 weight percent or more of the dispersoid forming component within the starting particulates.

40 14. The method of claim 11 wherein oxidizing the dispersoid forming component comprises forming a dispersoid, wherein about 95 weight percent or more of the base metal component is present in a reduced state.

15. The method of claim 11 wherein oxidizing the dispersoid forming component comprises forming a dispersoid with an average particle size of about 1 micron or less.

50 16. The method of claim 11 wherein forming the starting composition comprises selecting the base metal component from the group consisting of nickel, cobalt, iron, copper, and a combination thereof, and selecting the dispersoid forming component from the group consisting of hafnium, zirconium, yttrium, scandium, lanthanum, cerium, praseodymium, neodymium, promethium, samarium, europium, gadolinium, terbium, dysprosium, holmium, erbium, thulium, ytterbium, lutetium, and a combination thereof.

60 17. A method of forming a dispersoid hardened metallic material comprising:

forming a starting composition comprising a base metal component and a dispersoid forming component, wherein the base metal component comprises from about 50 weight percent to about 99.999 weight percent of the starting composition and the dispersoid forming component comprises from about 0.001 weight percent to about 1 weight percent of the starting composition;

fluidizing the starting composition with a fluidizing gas, wherein the fluidizing gas comprises an oxidizing agent partial pressure selected to preferentially oxidize the dispersoid forming component over the base metal component; and

5

preferentially oxidizing about 50 weight percent or more of the dispersoid forming component within the starting composition while the starting composition is in a solid state, wherein about 95 weight percent or more of the base metal component is present in a reduced state. 10

**18.** The method of claim 17 further comprising:

forming the starting composition into a starting powder having an average particle size of about 50 microns or less.

**19.** The method of claim 17, wherein:

15

preferentially oxidizing the dispersoid forming component comprises converting the starting powder into a dispersoid hardened metallic material; the method further comprising;

forming the dispersoid hardened metallic material into an 20 article.

**20.** The method of claim 17 wherein forming the starting composition comprises selecting the dispersoid forming component with an affinity to oxygen equal to or greater than that of aluminum. 25

\* \* \* \* \*